

## UNITED STATES PATENT OFFICE

HENRY J. LORANG, OF ST. LOUIS, MISSOURI, ASSIGNOR OF ONE-HALF TO FRANK J. KUNA, OF ST. LOUIS, MISSOURI

## METALLIC ALLOY

No Drawing. Application filed December 24, 1928. Serial No. 328,313.

This invention relates to an improved metallic alloy for use, more particularly, as a heating element for heating water by electricity.

The contemplated use of the heating element is in domestic radiators, in which each radiator will constitute a heating unit, the radiator being sealed and the same water being used over and over again.

10 My improved alloy is composed of the following ingredients used, as to each, in the percentage indicated:

|          | Per cent         |
|----------|------------------|
| Copper   | 1 $\frac{1}{8}$  |
| Zinc     | 1 $\frac{1}{8}$  |
| Tin      | 6 $\frac{1}{4}$  |
| Lead     | 2 $\frac{1}{4}$  |
| Antimony | 68 $\frac{3}{4}$ |

It is generally desirable to add about 1% more of zinc than indicated in the formula to allow for the loss which usually occurs when the zinc and copper are melted.

In addition to the metallic elements, there is added manganese dioxide and borax in the proportion of one-fourth of an ounce of each to to one pound of the mixed metals.

In preparing the alloy, the copper and zinc are first mixed and melted together, the resulting product being in the nature of brass. 20 The antimony and brass are then placed in a crucible containing the borax and manganese dioxide and melted, and the tin and lead are then added. I have found that the best results are secured when the tin and lead are 25 added to the other melted metals when the molten mass is at a temperature of about 1000° F.

Before using the borax, it is first melted down and allowed to harden and then ground and mixed with the manganese dioxide and the two are then mixed with the metals, either by being placed in the crucible in which the metals are melted, or by being mixed with the metals prior to placing them in the crucible. The borax acts as a flux and tends to prevent oxidation and consequent loss of antimony from the mixture. The manganese dioxide operates to render the alloy less brittle and less porous and, in general, acts to toughen the alloy. Neither the borax nor the

manganese dioxide form any appreciable combination with the metals, but they apparently act in the nature of catalytic agents to produce the results stated on the alloy. Both of them float on the melted mixture and prevent the formation of dross. In pouring the metal, a skimmer is used to hold the manganese dioxide and borax back as the melted alloy is poured from the container. A fresh quantity of manganese dioxide and borax may be used for each batch if desired, where large quantities are melted at a time; but where only small quantities, say, two or three pounds, of the alloy are melted at a time, the mixture of borax and manganese dioxide may be used for two or three meltings. Some impurities ultimately become mixed with the manganese dioxide and borax floating on top of the metallic batch, and for this reason, in commercial production in large quantities, it is desirable to use a fresh quantity of borax and manganese dioxide with each batch.

My improved heating element can be very cheaply produced, as compared with heating elements which have heretofore been employed, such, for instance, as those containing a large proportion of silver or tin. As heretofore employed, heating elements have been made in the form of wire wrapped around a core and hermetically enclosed in a casing. 80 They are relatively quite expensive, as, aside from the cost of labor in drawing the wire and constructing the heating elements, the alloy employed would probably cost in excess of \$1.00 a pound. As compared with these prior heating elements, my heating element can be produced very cheaply, the alloy, at the present price of metals, costing approximately fifteen cents a pound. My heating elements are cast in the form of bars and are, therefore, 90 very much cheaper to manufacture than heating elements necessitating drawing the alloy into the form of wire, then winding the wire around a core, enclosing it in a casing, etc.

Another advantage of my heating element is that, as shown by experiments conducted over a long period of time, it does not appear to be attacked by the water it is heating. For example, a heating element which had been in continuous use for 100 hours was calibrated 100

and it was impossible to discover the slightest diminution in its measurements.

Another very pronounced advantage of my improved heating element resides in the fact that owing to its composition, I find that the water can be brought to a given degree of heat, say, the boiling point, with the use of far less current than would be required to raise the water to such degree of heat with other heating elements, such as are now on the market. While not attempting to give a scientific explanation of this fact, it is my opinion that it is due to the presence in my alloy of a large percentage of antimony, as shown by the above formula, which metal, as known, ranks very low in the scale of conductors of electricity. There is also probably involved some phenomena having to do with the rapidity of heat interchange, as the heating element may be removed from boiling water and almost immediately taken in the hand, when it will be found to be only comfortably warm.

The alloy bars which I employ are preferably circular in cross-section, being about five-sixteenths of an inch in diameter and four inches in length. Other dimensions of the bars could, however, be employed.

While the manner of using the heating element is not involved in this application, it may be stated, in the interest of a full disclosure, that while my heating elements may be installed in the radiator, or other container of water to be heated, to act in the capacity of anodes and cathodes, respectively, I preferably install a number of my improved alloyed bars in a radiator or other metallic container of water and connect them in multiple to one side of the current and ground the container.

The proportions of the ingredients which I use in making my alloy as given above, I have found to give the best results. I do not wish, however, to be limited to the exact proportions indicated, as variations therewithin reasonable limits could be made without departing from the spirit of my invention. Irrespective of the exact proportions employed, an alloy constructed according to my invention would always be characterized by a preponderating quantity of antimony as compared with the other metals used. I believe also that no material departure from the formula could be advantageously made as respects the employment of equal parts of copper and zinc.

I claim:

1. A metallic alloy comprising the following metals combined in substantially the proportions stated, viz: copper,  $1\frac{3}{16}\%$ ; zinc,  $1\frac{3}{16}\%$ ; tin,  $6\frac{1}{4}\%$ ; lead,  $21\frac{3}{4}\%$ ; and antimony,  $68\frac{3}{4}\%$ .
2. The method of producing a metallic alloy, comprising a mixture of copper, zinc, lead and a preponderating quantity of

antimony which consists in melting the mixture in the presence of manganese dioxide and borax, the latter two elements being used in the proportion of approximately one-fourth of an ounce of each to one pound of the combined metals.

In testimony whereof, I have hereunto set my hand.

HENRY J. LORANG.

70

75

80

85

90

95

100

105

110

115

120

125

130